

## UNITED STATES PATENT OFFICE

2,406,575

## PREPARATION OF AN IMPROVED LUBRICANT

David W. Young, Roselle, N. J., and Harris D. Hineline, Mount Vernon, N. Y., assignors to Standard Oil Development Company, a corporation of Delaware

No Drawing. Application July 8, 1944,  
Serial No. 544,148

11 Claims. (Cl. 252—46.6)

1

This invention relates to thickened lubricants having an improved viscosity index; relates especially to thickened lubricants of improved viscosity index which have extreme pressure properties; and relates particularly to lubricants containing phosphorous pentasulfide treated, cyclized polymer such as polymethyl pentadiene.

A number of oil soluble substances have been found, which serve when dissolved in lubricants to thicken the lubricant and also to improve its viscosity index; that is, to reduce the rate of change of viscosity with change in temperature of the lubricant; among the best of which has been polyisobutylene. Polyisobutylene, however, lacks extreme pressure lubricating properties, and while the viscosity index of a lubricating oil containing polyisobutylene is excellent, it does not stand up well under conditions where lubrication of surfaces under extremely heavy pressure is required. On the other hand, various substances have been offered which contain such inorganic radicals as sulfur and chlorine which improve the extreme pressure properties of the lubricant, but do not sufficiently improve the viscosity index; and difficulty is encountered in adding both agents and obtaining satisfactory results.

The present invention provides a single soluble addition agent which, in a single substance, contains both V. I. improving elements and E. P. improving elements and is found to yield an excellent viscosity index, and, simultaneously, excellent extreme pressure properties.

For this purpose a polymerizable polyolefin such as 2-methyl pentadiene 1,3 is polymerized at low temperatures by the application of a Friedel-Crafts catalyst dissolved in a low freezing, non-complex forming solvent; to yield a high molecular weight polymer; which is then cyclized by the application of an appropriate cyclizing agent such as p-toluene sulfonic acid or aluminum bromide or stannic chloride or the like. The cyclized polymer is then treated at an elevated temperature with a compound of phosphorous and an element selected from the sulfur group. The preferred substance is phosphorous pentasulfide ( $P_2S_5$ ). Alternatively, other analogous compounds may be used, such for example as  $P_4S_3$ ,  $P_3S_6$ ,  $P_4S_5$  or  $P_2Se$  or  $P_4Se$  or  $P_2Se_3$ . This treatment adds into the cyclized polymer (or into the oil blend containing the cyclized polymer) a considerable quantity of combined sulfur (or selenium or tellurium) and a smaller quantity of combined phosphorous; which, together yield very effective extreme pressure properties while the high molecular weight of the cyclized poly-

mer yields the desired thickening and the desired improvement in viscosity index.

Thus the present invention provides a new composition of matter comprising a hydrocarbon solution of a cyclized polymer such as polymethyl pentadiene containing combined sulfur, and smaller or negligible quantities of combined phosphorous, dissolved in a hydrocarbon lubricant to yield a solution which remains liquid at low temperatures, and retains its body at relatively high temperatures. Other objects and details of the invention will be apparent from the following description.

The raw material for the present invention is a relatively high molecular weight polyolefinic polymer which is capable of cyclization. The preferred raw material is polymethyl pentadiene; that is the polymer of 2, methyl pentadiene-1,3 which polymerizes at low temperature quite readily into high molecular weight polymers, and when so polymerized cyclizes quite readily. Alternatively almost any of the other high molecular weight polyolefinic polymers are useful. Thus, such polyolefins as 2,5-methyl pentadiene-1,3 or 2-methyl-5-ethyl pentadiene-1,3 or the like are similarly useful. That is, substantially any of the polyolefins having more than 5 carbon atoms per molecule, in which there is an aliphatic substituent on the second carbon atom with a double linkage between the first and second carbon atom, is useful. Those compounds which are conjugated, that is, contain two double linkages separated by a single linkage, are preferred, but the condition of conjugation is not necessary. The limiting molecular size of the compounds is still unknown, but compounds as high as 12 or 14 carbon atoms per molecule are useful. All of these diolefins polymerize reasonably readily, cyclize readily, are soluble in hydrocarbons when polymerized and cyclized, and are reactive with phosphorous pentasulfide. Similarly, the triolefins including such substances as myrcene, having the formula



are very desirable raw materials, since they polymerize readily, cyclize readily, are oil-soluble when polymerized and cyclized, and combine readily with phosphorous pentasulfide after cyclization. Similarly, the triolefin known as allocycmene, having the formula



is equally advantageously useful. These sub-

stances are representative of polyolefins which polymerize at temperatures below 0° C. into oil soluble polymers having molecular weights above 3000, 4000 or 5000, up to several hundred thousand, with iodine numbers ranging from about 100 to 330 or above, which are readily cyclized to reduce the overall unsaturation, yet retain, in the cyclized condition, sufficient unsaturation to be reactive with phosphorous pentasulfide; and when so reacted, combine with the phosphorous and sulfur in such a way that the solubility in hydrocarbons remains good, the inorganic atoms are solidly held so that the compound is stable, yet the inorganic molecules are so placed as to result in an effective extreme pressure improvement.

Of these compounds, the polymer of methyl pentadiene is preferred.

In preparing this polymer, methyl pentadiene of good purity is used. In the examples herein-after given, a methyl pentadiene having a boiling point of 75° C. to 77° C. (at 760 mm. of Hg), a density of 0.7113 and an index of refraction  $N_D^{20}$  1.4472 was used. This material has a purity better than 95%, and further determinations indicate that its purity is in fact approximately 98%. The methyl pentadiene is cooled to a temperature about between 0° C. and -164° C. (preferably to a temperature between -40° C.) as set by liquid propane, and -103° C. as set by liquid ethylene. The methyl pentadiene by itself may be cooled, 30 by the application of a refrigerating jacket to the polymerization reactor. Alternatively the methyl pentadiene may be diluted with such substances as the lighter hydrocarbons or the alkyl, mono, or polyhalides or carbon disulfide or the like. Alternatively the methyl pentadiene may be cooled by an internal refrigerant-diluent. For this purpose such substances as liquid propane or liquid ethane or liquid ethylene or even liquid methane may be used; or the material may be cooled by solid carbon dioxide, or by dissolved liquid carbon dioxide; under vacuum if lower temperatures are desired.

The cold methylpentadiene is then polymerized by the application of a Friedel-Crafts catalyst which preferably is in solution in a low freezing noncomplex forming solvent. The Friedel-Crafts catalyst may be substantially any of the substances disclosed by N. O. Calloway in his article on "The Friedel-Crafts Synthesis" printed in the Journal of "Chemical Reviews," published for the American Chemical Society at Baltimore in 1935 in volume XVII, No. 3, the article beginning on page 327, the list being particularly well shown on page 375. These Friedel-Crafts active metal halides may be used as such in single salts, or may be used as double salts or complexes of several metals or several halides or even with alkoxy substituents. These catalysts may be solid, liquid or gaseous (boron trifluoride being gaseous; titanium tetrachloride being liquid; most of the remainder being solids). For solvent, the alkyl monohalides are preferred such as methyl or ethyl chloride. Other alkyl mono or polyhalides having melting points below 0° C. are also useful; as is carbon disulfide. All of these substances show an adequate solvent capacity for the Friedel-Crafts halides, especially aluminum chloride which is the preferred catalyst. Alternatively, and especially where catalyst complexes containing several halides, are used, the lighter hydrocarbons such as propane, butane, pentane, hexane, and the like may be used; the principal requirements being a solubility of at least 0.5% for

the active methyl halides and a freezing point below 0° C. (thereby being "low freezing").

The catalyst solution may be added to the cold olefinic material in any convenient manner which 5 will bring the catalyst solution quickly into intimate dispersion in the cold olefin. A convenient method is to spray the catalyst solution through a nebulizer on to the surface of the rapidly stirred cold olefinic material. Alternatively, the catalyst 10 solution may be jetted into a zone of high turbulence in the cold olefinic material such as the region near to a rapidly rotating propeller stirrer. Many other means for adding the catalyst are, however, available.

The reaction proceeds rapidly to yield the desired polymer, and the conversion may be carried to a yield of from 40-50% of the amount of methylpentadiene present, to a yield as high as 20 90-95%. Such high yields are, however, less desirable since the range of molecular weight is greater. When the reaction has reached the desired stage, the catalyst supply is interrupted. The solid polymer may be recovered in any desired manner; merely by boiling off residual unpolymerized methylpentadiene; and refrigerate 25 if present, or the reaction mixture may be treated with warm water or warm alcohol or warm naphtha, with or without small quantities of alcohol or the like.

The resulting polymer may have a molecular weight almost anywhere between 2000, 3000 or 12,000 and 30,000-100,000, depending upon the lowness of the polymerization temperature, the purity of the methylpentadiene, the presence and 30 purity of diluent-refrigerant, and the character of catalyst chosen. The preferred molecular weight is within the range between about 5000 and 35,000 to 45,000 since higher molecular weights break down somewhat more easily in 35 service and lower molecular weights require an undue amount of polymer to give a desirable amount of thickening.

After being brought up to room temperature, 40 the polymer is dried in any convenient manner and then is ready for the cyclization, which may be conducted in several ways. A preferred method is to put the polymer on the double roll mill at a moderate temperature, and mill into the polymer from 1% to 10% or 15% of p-toluene 45 sulfonic acid, continuing the milling until a thoroughly homogeneous mixture is obtained. The mixture is then removed from the mill and heated to a temperature approximately 100° C. for 30 to 60 minutes. This treatment effectively 50 cyclizes the polymer and by the cyclization reduces the iodine number to approximately 20 to 55 50. The polymer mixture may then be cooled to room temperature and is ready for the dissolving step.

60 Alternatively, the polymer may be dissolved in light naphtha and treated with stannic chloride at temperatures ranging from 20° C. to 80° C. for time intervals ranging from 15 minutes to 80 hours. This treatment also is effective for cyclization, and likewise reduces the iodine number to approximately 15 to 50.

70 Other methods which will be obvious to those skilled in the art may likewise be used for this cyclization step. The polymer is then ready for the phosphorous pentasulfide treatment.

The polymer is then dissolved in from 0.5% to 10% or 15% in the desired hydrocarbon lubricant. For the production of a fluid lubricant, a 75 high grade, well refined oil having a viscosity at

210° F. of from 30 S. S. U. to 70 S. S. U. may be used, sufficient polymer being dissolved in the oil to bring the viscosity and viscosity index to the desired values. Alternatively, if a heavy grease is to be made, a much heavier lubricant stock may be utilized and the various addition agents used to make heavy greases may be incorporated; together with from 1% to 15% or 20% of the polymer.

To this solution there is then added a substantial quantity of phosphorous pentasulfide, the amount ranging from 1% to 10% or 15% of the amount of cyclized polymer. The oil solution is then heated to temperatures ranging from 150° C. to 225° C. for from 15 minutes to 150 minutes. The solution is then filtered to remove any uncombined phosphorous pentasulfide, and any insoluble reaction products, the material being preferably filtered while hot because of the more rapid filtering rate. In the preparation of greases it is, of course, desirable that the auxiliary components be added after the filtration step.

The above outlined procedure applies particularly to methylpentadiene, and to its polymers, but substantially the same procedure may be applied to a wide range of polymerizable substances, polymers, and high molecular weight substances in general, it being merely necessary that they be capable of cyclization; when cyclized be soluble in hydrocarbons, and when cyclized retain a sufficiently high iodine number, and a sufficient amount of unsaturation to combine with the phosphorous pentasulfide.

Thus, for instance, an interpolymer of isobutylene with a polyolefin having more than 5 carbon atoms in which a substantial quantity of the polyolefin is interpolymerized, is similarly useful, especially with polyolefins up to 12 or 14 carbon atoms per molecule and especially when the quantity of polyolefin interpolymerized is substantial in amount. That is, it is desirable that the iodine number of the cyclized polymer be above 5, and it is also essential that the cyclized polymer be oil-soluble. This latter requirement eliminates the polymers of simple butadiene, isoprene and pentadiene and copolymers containing substantial portions of butadiene.

It is further essential that to be useful, the polymers must cyclize with a minimum of cross linkages, which is found to be a characteristic of the polyolefins having more than 5 carbon atoms, but not a characteristic of butadiene, and the presence of butadiene per se to the extent of more than about 20% introduces so much cross linkage upon cyclization as to render the cyclized polymer useless. Thus, copolymers of isobutylene with butadiene or isoprene or piperylene, containing from 2% to 15% or 20% of butadiene are usable. Copolymers of isobutylene with dimethyl butadiene, myrcene, dimethylallyl and the like, up to 12 or 14 carbon atoms, are usable, especially when the proportion of interpolymerized diolefins exceeds 5% or 10%. Likewise, as will be evident from the above description, these polyolefins may be used with any proportion of isobutylene, down to 0.

It may be noted that the phosphorous pentachloride treatment of the cyclized polymer introduces sulfur into the molecule without the establishment of any cross linkage, differing in that respect from vulcanization, which introduces a maximum of cross linkages into the compound between adjacent molecules. It may be noted that the introduction of cross linkages destroys the oil-solubility, whereas the introduc-

tion of sulfur without cross linkages retains the oil-solubility and it is of the essence of the present invention that, broadly, the polymer is cyclized and sulfurized without the introduction of cross linkage, in order to obtain a compound of high molecular weight which contains substantial quantities of combined sulfur (the effect of which is aided by the presence of smaller quantities of phosphorous) and accordingly, the invention is applicable to any polymer which can be cyclized and combined with phosphorous pentasulfide without the formation of sufficient cross linkages to destroy the solubility in hydrocarbons.

*Example 1*

Approximately 100 parts of methyl pentadiene having a purity of approximately 95% were cooled to a temperature of approximately -88° C. by the addition thereto of approximately 300 parts of liquid ethane. The mixture was then polymerized by the addition of approximately 50 parts of a solution of aluminum chloride in ethyl chloride having a concentration of approximately 2%, the catalyst solution being sprayed on to the surface of the rapidly stirred olefinic mixture. The polymerization proceeded quickly to yield a solid polymer having a molecular weight of approximately 40,000. The polymerization mixture was thrown into hot water to volatilize residual refrigerant and to separate unpolymerized methyl pentadiene. The yield was approximately 80%. The polymer was then placed on the double roll mill, washed with water until most of the residual traces of catalyst were removed, and then approximately 3 parts by weight (per hundred of polymer) of p-toluene sulfonic acid were added and thoroughly milled into the solid polymer. The milling was continued until a thoroughly homogeneous mixture was obtained. The solid mixture was then placed in a hot air oven at 100° C. for 30 minutes.

The mixture was then cooled and approximately 50 parts by weight of the polymer were dissolved in 1000 parts by weight of a high grade 45 paraffinic mineral lubricating oil which had a viscosity at 210° F. of 52 S. S. U. and a V. I. of 98. When the solution was complete, yielding a clear fluid solution, approximately 50 parts by weight of powdered yellow phosphoric pentasulfide  $P_2S_5$  was added, well stirred in and the mixture heated to a temperature of 180° C. for 30 minutes, the mixture being well stirred during the heating step. At the end of the 30 minutes, the mixture was cooled to approximately 25° C. and filtered 55 through a paper filter to yield a clear filtrate.

Chemical analysis of the clear filtrate showed that it contained 0.58% of phosphorous and 2.03% of sulfur.

Viscosity determinations and viscosity index 60 determinations showed the following inspection results:

|    | S. S. U. vis.<br>cosity at 100°<br>F. | S. S. U. vis.<br>cosity at 210°<br>F. | V. I. |
|----|---------------------------------------|---------------------------------------|-------|
| 65 | 488                                   | 74                                    | 131   |

These results show that the resulting oil has 70 an excellent viscosity and an excellent viscosity index.

Other portions of this oil product were then charged into the Almen machine for the usual 30 second run. At the end of the 30 seconds, the successive 2 lb. weights were added at 10 second inter-

vals until the full number of 15 weights had been added. The oil carried all 15 weights. The pin and bushing were made of steel and at the end of the test the pin and bushing were in good condition.

*Example 2*

A mixture was prepared consisting of approximately 100 parts by volume of methyl pentadiene having a purity of approximately 98% and 400 parts of liquid ethylene. The presence of the liquid ethylene cooled the material to a temperature of approximately  $-103^{\circ}$  C. This mixture was then polymerized by the addition of approximately 75 parts by volume of a solution of aluminum chloride in methyl chloride in a concentration of approximately 0.8%. The polymerization was conducted by spraying the catalyst solution onto the surface of the rapidly stirred olefinic material. The polymerization proceeded rapidly to yield a solid polymer having a molecular weight (by the Staudinger method) of approximately 44,000. The polymerization mixture was then thrown into warm water to volatilize residual traces of refrigerant and to separate out any unpolymerized methyl pentadiene. The yield of polymer was approximately 69%. The solid polymer was then placed on a double roll mill and washed with water until most of the residual traces of catalyst and monomer were removed. When this stage was reached, approximately 10 parts by weight (per 100 of polymer) of p-toluene sulfonic acid were added and thoroughly milled into the solid polymer. The milling was continued until a thoroughly homogeneous mixture was obtained. The mixture was then placed in a hot air oven at  $100^{\circ}$  C. for 20 minutes. The brown polymer mixture was then cooled and approximately 50 parts by weight of the polymer were dissolved in 1000 parts by weight of a good lubricating oil which had a viscosity at  $100^{\circ}$  F. of 128 S. S. U., a viscosity at  $210^{\circ}$  F. of 42 S. S. U. and a V. I. of 109. When the solution was about complete, approximately 50 parts by weight of powdered yellow phosphorous pentasulfide (P<sub>2</sub>S<sub>5</sub>) was added and well stirred in. The mixture was then heated to a temperature of  $180^{\circ}$  C. for 60 minutes, the mixture being well stirred during the heating period. At the end of the 60 minutes the mixture was cooled to approximately  $35^{\circ}$  C. and filtered through a paper filter to remove residual traces of uncombined phosphorous pentasulfide and to yield a clear filtrate. The filtrate was then blown with air, using about 5 cubic feet per hour per kilo of solution for a period of 2 hours to remove traces of hydrogen sulfide and to deodorize the oil.

Chemical analysis of the clear, odorless filtrate showed that it contained 0.8% of combined phosphorous and 2.88% of combined sulfur. Viscosity determinations and viscosity index determinations showed the following inspection results:

| S. S. U. at<br>$100^{\circ}$ F. | S. S. U. at<br>$210^{\circ}$ F. | V. I. |
|---------------------------------|---------------------------------|-------|
| 284                             | 68                              | 134   |

These determinations show that the resulting oil has an excellent viscosity and an excellent viscosity index.

Portions of this oil were then charged into the Almen machine for the shock loading test. All 15 weights (2 lbs. each) were placed on the arm and allowed to drop simultaneously. The oil car-

ried all 15 weights under this shock loading and after the test the pin and bushing, which were made of steel, were in good condition.

The oil was then tested under gradual loading conditions in the Almen machine as outlined in Example 1. The cyclized P<sub>2</sub>S<sub>5</sub> treated polymer in solution in the oil carried all 15 weights.

These results indicate that the oil prepared as above described is a high grade lubricant having a very advantageous viscosity index and a very valuable extreme pressure property.

While there are above disclosed but a limited number of embodiments of the invention, it is possible to provide still other embodiments without departing from the inventive concept herein disclosed and it is, therefore, desired that only such limitations be imposed upon the appended claims as are stated therein or required by the higher art.

20 The invention claimed is:

1. An improved lubricant comprising a hydrocarbon lubricating agent having dissolved therein .5 to 20% of polymer of a polyolefin having more than 5 carbon atoms per molecule which is characterized by cyclization and the presence of phosphorous sulfide.

2. An improved lubricant comprising in combination a hydrocarbon material and a solute therein comprising .5% to 20% of a cyclized, phosphorous pentasulfide treated, polymer of a polyolefin having 6 to 14 carbon atoms per molecule, a molecular weight between 3,000 and 100,000 and an iodine number after cyclizing between 5 and 50.

3. An improved lubricant comprising in combination a hydrocarbon oil and solute therein comprising .5 to 20% of a cyclized, phosphorous pentasulfide treated, polymer of methyl pentadiene.

4. An improved lubricant comprising in combination a hydrocarbon oil and a solute therein comprising .5 to 20% of a cyclized, phosphorous pentasulfide treated, polymer of 2-methyl pentadiene-1,3.

45 5. An improved lubricant comprising in combination a hydrocarbon oil and a solute therein comprising .5 to 20% of a cyclized, phosphorous pentasulfide treated, polymer of myrcene.

6. An improved lubricant comprising in combination a hydrocarbon oil and a solute therein comprising .5 to 20% of a cyclized, phosphorous pentachloride treated, polymer of allo-octyne.

7. The method of preparing a lubricant comprising the steps in combination of polymerizing 55 a polyolefin having from 6 to 14 carbon atoms per molecule, cyclizing the polymer, treating the cyclized polymer with a compound of phosphorous and an element from the sulfur group and dissolving .5 to 20% of the cyclized phosphorous compound treated polymer in a lubricating material.

8. The method of preparing a lubricant comprising the steps in combination of polymerizing a polyolefin having from 6 to 14 carbon atoms per molecule, cyclizing the polymer, dissolving the cyclized polymer in a hydrocarbon liquid, treating the cyclized polymer with a compound of phosphorous and an element from the sulfur group and dissolving .5 to 20% of the cyclized phosphorous compound treated polymer in a lubricating material.

9. The process of preparing a lubricant comprising the steps in combination of polymerizing a methyl pentadiene, cyclizing the methyl pentadiene, dissolving .5 to 20% of the cyclized

methyl pentadiene in a hydrocarbon lubricant, and treating the dissolved polymer with phosphorous pentasulfide.

10. The process of preparing a lubricant comprising the steps in combination of polymerizing a methyl pentadiene, cyclicizing the methyl pentadiene by the application thereto of p-sulfonic acid, dissolving .5 to 20% of the cyclicized methyl pentadiene in a hydrocarbon lubricant, and treating the dissolved polymer with phosphorous pentasulfide. 10

11. The process of preparing a lubricant comprising the steps in combination of polymerizing a methyl pentadiene, cyclicizing the methyl pentadiene by the application thereto of stannic chloride, dissolving .5 to 20% of the cyclicized methyl pentadiene in a hydrocarbon lubricant and treating the dissolved polymer with phosphorous pentasulfide.

DAVID W. YOUNG.  
HARRIS D. HINELINE.